

## UNITED STATES PATENT OFFICE

2,322,001

## METHOD OF PRODUCING DYE IMAGES

George Ehrenfried, Rochester, N. Y., assignor to  
 Eastman Kodak Company, Rochester, N. Y., a  
 corporation of New Jersey

No Drawing. Application October 10, 1940,  
 Serial No. 360,622

6 Claims. (Cl. 95—6)

This invention relates to a method for producing colored photographic images and particularly to a method of forming colored images in the bleach-out process of color photography.

Christensen U. S. Patent 1,517,049, November 25, 1924 describes a process for producing a dye image in which a dyed gelatin layer containing a silver image is treated with a solution of a strong reducing agent such as sodium hydrosulfite or stannous chloride. The reducing bleach bath destroys the dye in the layer selectively in the region of the silver image, giving a positive dye image from a negative silver image. The destruction of a dye to form a photographic image in this process appears to depend upon the catalytic action of the silver image which results in the destruction of the dye in that portion of the film when treated with a suitable reducing bleach bath.

I have found that in many cases the image-forming dyes used in this process may be more readily bleached if a silver salt image is used in place of a metallic silver image and the bleaching bath is allowed to reduce this silver salt to metallic silver in the same operation as the destruction of the dye. The silver salt image may be produced, for example, by rehalogenizing a developed and fixed silver image.

It is, therefore, an object to provide a novel method of forming a colored photographic image in a photographic layer. A further object is to provide a novel method for destroying a dye uniformly dispersed in a photographic layer under the influence of a silver salt image.

These objects are preferably accomplished according to my invention by developing the emulsion layer containing the uniformly dispersed image-forming dye, fixing, washing, and then rehalogenizing the silver image thus formed and treating the layer with a suitable reducing bleach bath.

The photographic element treated according to my invention may comprise a single emulsion layer or a plurality of emulsion layers coated on one or both sides of a suitable support. This support may be a cellulosic material such as pigmented cellulosic material or paper. The emulsion layer or layers may contain a uniformly dispersed dye prior to exposure or a dye intermediate in which a colored compound may be formed after exposure. I prefer to use the general class of poly-azo dyes as disclosed in Christensen U. S. Patent 1,517,049, though not necessarily the same dyes.

If a three-layer photographic element is used for the production of natural color images, the three emulsion layers preferably contain dyes

each of which is roughly complementary in color to the effective sensitivity of the emulsion layer. The red sensitive layer may be colored blue-green with one of the following dyes.

5 *Example 1.*—Pontamine Fast Green 5BL (Du Pont).

*Example 2.*—A blue dye of less suitable color, but of satisfactory bleaching properties, made by tetrazotizing 4,4'-diamino-2,2'-dimethyl, 5,5'-dimethoxy triphenylmethane and coupling it with two mols of chromotropic acid.

*Example 3.*—Indigo.

The green-sensitive layer may be colored magenta with one of the following dyes, some of which are described in Seymour, Young, and Chechak U. S. patent application Serial No. 333,808, filed May 7, 1940.

10 *Example 4.*—Monosol Carmine LS (Color Index No. 357).

20 *Example 5.*—A dye made by tetrazotizing 4,4'-diamino-3,3'-dimethoxy diphenyl methane and coupling with 2 mols of R-salt.

15 *Example 6.*—The dye made by tetrazotizing 1 mol of 4,4'-diamino triphenyl methane and coupling with 2 mols of N-lauroyl H-acid.

25 *Example 7.*—The dyes made by tetrazotizing 1 mol of 4,4'-diamino-3,3', 6,6'-tetramethyl triphenyl methane and coupling with 2 mols of N-heptyl H-acid or one of the following compounds:

30 *Example 8.*—N-lauroyl H-acid.

*Example 9.*—N-benzoyl H-acid.

*Example 10.*—1-naphthol-3,6-disulfonic acid-3-β-naphthalene sulfonate.

35 *Example 11.*—N(naphthalene - β - sulfonyl) H-acid.

*Example 12.*—N(4-benzamido benzoyl) H-acid.

*Example 13.*—Chromotropic acid.

40 *Example 14.*—The dye made by tetrazotizing 4,4'-diamino-2,2'-dimethyl-5,5'-dimethoxy triphenyl methane and coupling with 2 mols of 1-naphthol-8-para-tolyl sulfonate-3,6-disulfonic acid.

45 *Example 15.*—The dye made by tetrazotizing 4,4'-diamino-2,2',5,5'-tetramethoxy triphenyl methane and coupling with 2 mols of R-acid. The blue sensitive layer may be colored yellow with a suitable diazo dye such as the following, some of which are described in Carroll & Chechak, U. S. patent applications 333,806 and 333,807, filed May 7, 1940.

50 *Example 16.*—The dye made by tetrazotizing Pontamine Diazo Yellow 2GL and coupling with 2 mols of 2-chloro-5-hydroxy toluene or one of the following compounds:

55 *Example 17.*—p-Cresol.

*Example 18.*—2,4-dimethyl phenol.

*Example 19.*—The dye made by tetrazotizing 4,4'-diamino-3,3'-dimethyl-4''-methoxy triphenylmethane-3''-sulfonic acid and coupling with 2 mols of naphthionic acid.

*Example 20.*—The dye made by diazotizing 2-naphthylamine-4,8-disulfonic acid, coupling with meta-toluidine and treating the product with phosgene.

*Example 21.*—The dye made by tetrazotizing benzidine and coupling with 2 mols of phenol p-sulfonic acid.

*Example 22.*—The dye made by tetrazotizing 4,4'-diamino stilbene disulfonic acid, coupling with 2 mols of phenol and forming the di-n-propyl ether of the product.

*Example 23.*—The dye made by tetrazotizing 4,4'-diamino stilbene disulfonic acid, coupling with 2 mols of phenol and forming the dibutyl ether of the product.

*Example 24.*—The dye made by tetrazotizing 4,4'-diamino stilbene disulfonic acid, coupling with 2 mols of 2,6-dimethyl phenol and forming the di-n-propyl ether of the product.

The layers need not be colored complementary to their sensitivity, however, but may be colored alternatively with a dye that transmits the color for which the layer is mainly sensitive.

This film is exposed in a camera or under a suitable color positive or negative. For example, it may be exposed to a natural color transparency by a single exposure to tungsten light through suitable correcting filters or by three simultaneous or successive exposures to light transmitted by red, green and blue filters in a suitable ratio of times or intensities. It is then developed in an ordinary black and white developer, washed, and fixed. The silver image is then reconverted to a silver halide such as silver chloride and the dyes are bleached by treatment in a sodium stannite or sodium hydrosulfite bleach bath. This reduces the silver halide image to metallic silver, and during the same operation, destroys the dye in the region of the silver image so formed. The film is then again washed and the silver image is reconverted to silver halide in the same solution previously used for this purpose or in any other suitable bath. The film is then fixed in hypo to remove the silver halide and is washed and dried leaving pure dye images in the layers.

A specific method of treating a three-layer photographic element according to my invention will now be described.

A multi-layer element having coated on a suitable support a red-sensitive layer containing Pontamine Fast Green 5BL, a green sensitive layer containing the dye made by tetrazotizing 4,4' - diamino - 2,2',5,5' - tetramethyl triphenyl methane and coupling with 2 moles of N-heptoyl "H-acid" and a blue-sensitive layer containing the dipropyl ether of Brilliant Yellow (Color Index No. 364) is exposed to a natural color transparency by a single exposure to tungsten light through suitable correcting filters. The element is then developed for about eight minutes at 68° F. in a tank of the following developer:

Monomethyl-p-aminophenol  
sulfate \_\_\_\_\_ grams 2  
Hydroquinone \_\_\_\_\_ do 5  
Sodium sulfite (desiccated) \_\_\_\_\_ do 100  
Borax, granular \_\_\_\_\_ do 20  
Water to \_\_\_\_\_ liter 1

The print is now placed for two minutes in a stop bath consisting of: acetic acid, 28%, 500 c.c.; water, 4 liters.

The film is then thoroughly fixed in acid hypo of the following composition:

Water (about 125° F.) \_\_\_\_\_ c.c. 600  
Hypo \_\_\_\_\_ grams 240  
5 Sodium sulfite \_\_\_\_\_ do 15  
Acetic acid (28%) \_\_\_\_\_ c.c. 48  
Boric acid crystals \_\_\_\_\_ grams 7.5  
Potassium alum \_\_\_\_\_ do 15  
Water to \_\_\_\_\_ liter 1

10 The element is again washed and may then be hardened in a 1 to 20 formalin solution, although this hardening step may be omitted if the emulsions have been suitably hardened before coating.

15 The silver images produced by the development are bleached to silver chloride by treatment for about ten minutes in the following solution:

20 Cupric chloride \_\_\_\_\_ grams 100  
Hydrochloric acid concentrated \_\_\_\_\_ c.c. 25  
Water to \_\_\_\_\_ liter 1

25 The film is then washed for about 5 minutes in several changes of distilled water. The dyes are then bleached by treatment for about five minutes in a sodium stannite solution made in the following manner:

30 Stannous chloride \_\_\_\_\_ grams 8  
Water (distilled) \_\_\_\_\_ c.c. 100  
Sodium hydroxide (10% solution) \_\_\_\_\_ do 100

35 The element is again washed first in plain water for about 30 seconds and then for 5 minutes in a solution of 20 c.c. concentrated hydrochloric in 1 liter of water. The silver images are then bleached in the same copper chloride bath previously used. This reconverts to silver chloride the silver formed in the bleaching bath by reduction with the sodium stannite solution, to silver chloride. The film is then again washed and is then fixed in an acid hypo bath of the same composition as that previously used. It is then washed and dried.

40 45 In place of the copper chloride bleach bath used to bleach the silver images to silver chloride, baths of the following composition may be used:

A. Quinone, hydrochloric acid and ethyl alcohol.

50 B. Ferric chloride and hydrochloric acid.  
C. Ammonium persulphate and hydrochloric acid.

55 In some cases it is desirable to add an organic solvent to the sodium stannite bleach bath to reduce highlight stain. One volume of tertiary butyl alcohol to about 10 volumes of the bleach bath appears to be a satisfactory solvent for this purpose.

60 With certain dyes, Pontamine Fast Green 5BL for example, a 2% solution of sodium hydrosulfite can be used to bleach the dyes in the presence of the silver chloride image.

65 A photographic element containing the dyes referred to above may be processed according to the method of the present invention to form colored images giving satisfactory color reproduction. Many of the image forming dyes which we propose to use bleach poorly when treated with a reducing bleach bath in the presence of a silver image but may be successfully bleached by these baths in the presence of a silver halide image. However, I have found that, while the sodium stannite or alkaline sodium hydrosulfite bleach baths can be used to bleach the dyes with simultaneous reduction of a silver chloride image pro-

duced from a developed and fixed silver image, I have not found it possible to use these bleaches to develop the original latent image and thus effect development and bleaching in one operation.

Other modifications of the invention will be apparent to those skilled in the art and it is to be understood that my invention is to be taken as limited only by the scope of the appended claims.

I claim:

1. The method of forming a colored image in a photographic layer containing a bleachable azo dye uniformly dispersed therein and a rehalogenized silver image, which comprises bleaching the dye in the region of said image with an alkaline stannous chloride bleach bath.

2. The method of forming a colored image in a photographic layer containing a bleachable azo dye uniformly dispersed therein and a rehalogenized silver image, which comprises bleaching the dye in the region of said image with a sodium hydrosulfite bleach bath.

3. The method of forming a colored image in a photographic layer containing a bleachable azo dye and unexposed silver halide uniformly dispersed therein, which comprises exposing and developing said layer, removing the unexposed silver halide without affecting the silver image formed by development, reconverting the silver image to silver halide, and bleaching the dye in the presence of said image with alkaline stannous chloride to form a colorless dye compound and leave unaffected the dye in the remaining portions of the layer.

4. The method of forming a colored image in a photographic layer containing a bleachable azo dye and unexposed silver halide uniformly dis-

persed therein, which comprises exposing and developing said layer, removing the unexposed silver halide without affecting the silver image formed by development, reconverting the silver image to silver halide, and bleaching the dye in the presence of said image with sodium hydrosulfite to form a colorless dye compound and leave unaffected the dye in the remaining portions of the layer.

5. The method of forming a colored image in a photographic layer containing a bleachable azo dye and unexposed silver halide uniformly dispersed therein, which comprises exposing and developing said layer, removing the unexposed silver halide without affecting the silver image formed by development, reconverting the silver image to silver halide, and bleaching the dye in the presence of said image with a stannite of an alkali-metal to form a colorless dye compound and leave unaffected the dye in the remaining portions of the layer.

6. The method of forming a colored image in a photographic layer containing a bleachable azo dye and unexposed silver halide uniformly dispersed therein, which comprises exposing and developing said layer, removing the undeveloped silver halide without affecting the silver image formed by development, reconverting the silver image to silver halide, and bleaching the dye in an alkaline, reducing bleach bath comprising an alkali metal salt of an acid selected from the group consisting of stannous acid and hydrosulfurous acid and free of silver halide developing agent in the presence of said image to form a colorless dye compound and leave unaffected the dye in the remaining portions of the layer.

GEORGE EHRENFRIED.